

Feb. 25, 1930.

T. MIDGLEY, JR

1,748,518

COOLING DEVICE FOR VALVES AND THE LIKE

Filed Jan. 10, 1918



Fig. 2.

Fig. 3.

Fig. 1.

WITNESSES.

*Walter D. Biggs*  
*Warren Schmidling*

INVENTOR  
*Thomas Midgley Jr.*  
BY  
*Kerr, Page, Cooper & Haynard*  
ATTORNEY

Patented Feb. 25, 1930

1,748,518

# UNITED STATES PATENT OFFICE

THOMAS MIDGLEY, JR., OF DAYTON, OHIO, ASSIGNOR, BY MESNE ASSIGNMENTS, TO  
DELCO LIGHT COMPANY, OF DAYTON, OHIO, A CORPORATION OF DELAWARE

## COOLING DEVICE FOR VALVES AND THE LIKE

Application filed January 10, 1918. Serial No. 211,224.

The present invention relates to improvements in the construction and manufacture of parts of cooling systems or devices in which the transfer of heat from one metallic body 5 to another body is relied upon to produce the desired cooling effect.

As an instance of one particular form of application of such invention, the present description relates to valves of internal combustion engines, which valves are hollow and contain a small amount of "working" mercury, which vaporizes in contact with the heated portion of the valve and condenses in the cooling portion of the valve. Devices 0 of this character are set forth in the application of C. F. Kettering, Serial No. 211,156, filed January 10, 1918, patented March 27, 1928, Patent No. 1,663,709, which describes and illustrates a valve or other engine part 0 having a body which is subjected to the heat of engine operation, and is formed with a chamber containing a small quantity of working mercury, portions of which, when vaporized by the heat, pass up the hollow 5 stem of the valve, are there cooled and returned to the bottom of the valve, which process cools the valve head.

As described more in detail in said Kettering application Ser. No. 211,156, the interior 0 of the valve may be provided with heat dissipating or transferring surfaces or bodies, which may be an amalgam coating or veneer applied to the interior wall of the hollow valve. This coating or veneer appears to 5 have the effect of facilitating the transfer of the heat from the metal of the valve to the working mercury, and vice versa. As a result, the mercury is raised to its boiling point more rapidly than would be the case without any such amalgam coating, and begins to function to cool the valve earlier, and before the valve reaches an extremely high temperature. Moreover, when the working mercury is functioning to cool the valve, this veneer or coating acts as an effective intermediary to transfer the heat from the vaporized mercury to the metal of the cooling part of the valve, thereby cooling or condensing the vaporized mercury and aiding still further in dissipating the heat.

Among the objects of the present invention are to provide devices of this character with bodies, or a coating, or a veneer, of heat transferring medium which will have marked qualities of heat conduction, mechanical 55 strength, ability to stand up under the high temperature conditions to which the device is subjected, as well as mechanical vibration, while employing only relatively inexpensive means for attaining these results. Further 60 objects of the invention will be obvious from the ensuing description.

In order that the invention may be clearly comprehended, reference will now be made to the accompanying drawing which illustrates a preferred embodiment of the invention as applied to the valves of internal combustion engines.

In said drawing:

Fig. 1 shows in cross section a valve to 70 which the present invention is applied.

Figs. 2 and 3 illustrate the method of hermetically sealing the valve.

Referring to Fig. 1, the steel valve here illustrated comprises the head portion 10 and 75 a stem 12, which may be provided with radiating fins or ribs 13, slipped over the stem in any suitable manner. The head portion 10 may be welded to the stem 12, so that the head and stem will constitute substantially 80 one continuous piece of metal.

In the interior of the hollow stem is provided the small portion of so-called "working" mercury 20, which vaporizes during the 85 operation of the valve. The vapor passes up towards the top of the stem, where it is cooled and again transformed into its liquid state, dropping by gravity to the bottom of the stem, thus setting up a continuous or cyclic 90 automatic cooling action.

The inner wall of the stem is provided, as shown, with an intermediate heat transferring medium indicated by the reference number 14, which forms a coating, veneer or body superposed upon and in intimate contact with the inner face of said stem chamber for the purpose of facilitating the transfer of heat 95 between the wall and the mercury, and vice versa. This coating is purposely shown on 100

an exaggerated scale in the drawing to facilitate the understanding of the invention.

The operation and efficacy of the valve can be considerably increased by using such an intermediate heat transferring medium, which consists of an amalgam or alloy of mercury, applied in the form of a permanent coating before the valve is placed in use. Such an intermediate medium presents a surface which can be "wetted" by the working mercury and has marked advantages, in facilitating the transfer of heat between the wall and the mercury, which appear to be absent when the working mercury is in contact with a surface which it can not wet.

My improvements are directed first toward the securing of the best kind of amalgam for such a coating. My preferred forms of coating are devised both with reference to ability to facilitate transfer of heat, and ability to adhere strongly and permanently to the steel of the wall which supports it, so as to form a structure or coating which is mechanically strong and will not break off or become detached as a result of the vibration and temperature conditions under which the valve operates. These conditions are best met by the use of an amalgam, including a metal such as iron, which will strongly adhere to the metal of the valve; in an amalgam of this character, the mercury of the amalgam facilitates transfer of heat to and from the working mercury, while the iron of the amalgam facilitates transfer of heat to and from the steel of the valve, so that the metals of the amalgam, so to speak, form a link or chain system for the easy transfer of heat between the parts.

I have also discovered another characteristic which gives added efficiency to such an intermediate heat transferring medium, viz., that it should be made of material which will not only tend to adhere strongly to the steel of the valve, but which, in the event of any part of the amalgam becoming disassociated from the steel, will also reassociate itself and adhere strongly to the steel that may have become exposed. That is, if the amalgam "breaks down", (that is, disassociates itself from the steel,) the coating or veneer becomes automatically renewed without having to replace it or recoat it by an external operation. This property of renewal or re-coating under operating conditions is hereinafter referred to as the "building up" property of the amalgam. I have found that excellent results are to be obtained in practice by employing an intermediate heat transfer medium consisting of an iron amalgam with tin, or such equivalents as lead, or both tin and lead together. I prefer to use an iron amalgam containing thirty per cent (30%) tin lead, which latter serves to protect the iron in the amalgam as above described, and is coated or plated on to the inner walls of the

stem chamber in any suitable manner. In the use of amalgams containing tin or such an equivalent as lead, or both, when any of the amalgam of the veneer breaks down under operating conditions it becomes mixed with the working mercury of the valve, and is carried by the mercury vapor back into contact with that portion of the steel from which the coating became detached, and thereby builds up or renews the coating at the desired point. The best results achieved up to this time have been by the use of an iron amalgam which also contains metals with building up properties, such as tin and lead.

I also obtain improved results by placing a small quantity of an amalgam having "building up" properties in the working mercury, which amalgam is carried by the heated mercury into contact with any exposed part of the steel of the stem, with which it adheres. This amalgam which is mixed with the working mercury may be the same as that which forms the coating or veneer, or it may be one of the components of said coating or veneer. In practice, I prefer to use a tin or lead amalgam, or a tin-lead amalgam mixed with the working mercury, and I have obtained excellent results by the use of a tin or tin-lead amalgam mixed with the working mercury in the proportion of 30 to 50 per cent of the amalgam, in conjunction with a 30% to 50% tin-lead amalgam coating or veneer.

It will be understood that the proportion of tin-lead present in the working mercury due to the introduction of previously prepared tin-lead amalgam or to the introduction of tin-lead directly, is susceptible of considerable variation, and may vary from nothing as in the case of pure working mercury over a great range as described herein. It will be apparent from the foregoing that I prefer to use "building up" amalgam in both the veneer and the working mercury, though this is not necessary since such amalgam, whether originally introduced into the working mercury or originally applied to the stem and subsequently broken loose from the steel, will be eventually carried by the working mercury into contact with any exposed part of the steel to which it will adhere.

In some cases I may use a veneer consisting of a simple iron amalgam, plated or otherwise applied. The iron of the amalgam will adhere very strongly to the steel of the stem. While iron tends to adhere more strongly to the steel than other metals, such coatings consisting of mercury and iron alone are not quite so satisfactory as some of the other amalgams mentioned which contain tin or lead, on account of the lack on the part of the simple iron amalgam, of the property of "building up" as described above. By using an amalgam of iron with tin or lead or both, the valuable properties of the iron in adher-

ing to the steel and facilitating the transmission of heat from the veneer 14 to the steel stem are retained, while the valuable "building up" properties of the amalgam, due to the presence of the tin or lead insure the permanence of the coating in use.

I have also found that I am able to obtain satisfactory results by the use of a veneer 14 of tin applied in any suitable manner to adhere to the steel; this tin becomes transformed into a tin amalgam when the valve has been in use, as a result of the action of the working mercury on the tin.

I may also use an amalgam veneer 14, for instance, iron amalgam, for the valve stem, and place in the working mercury a quantity of another amalgam, which may have "building up" properties, for instance, tin-lead amalgam, relying upon the action of the working mercury to carry the tin-lead amalgam to the iron amalgam veneer so as to build it up continuously. The tin-lead amalgam is preferably present in the working mercury in such quantity that the proportion of tin-lead therein is between 30% to 50%.

The thickness of the coating or veneer may vary in practice; I find that a relatively thin layer is quite sufficient for the purposes of the invention.

30 The working mercury may in some cases be replaced by a tin or lead amalgam, or tin-lead amalgam, which, on account of its low boiling point, is able to act as a heat transfer medium in a manner somewhat similar to the working mercury; or the inside walls of the valve may be provided with an amalgam coating, employing an amalgam such as described above, without the presence of the working mercury, and the valve will be thereby cooled to a certain extent; but I find it always preferable to use the working mercury along with the amalgam.

45 The methods of applying the amalgam coating or veneer 14 to the valve stem are fully described and claimed in my divisional application Serial No. 256,530, filed October 4, 1918 patented July 15, 1924, Patent Number 1,501,862. After the valve stem has been provided with its amalgam coating, as there- 50 in described or in any other preferred manner.

The working mercury is introduced into the valve in the desired quantity, (for example, about five grams), and if it is desired to employ a quantity of amalgam for the purpose of building up the coating or veneer in the manner herein described, then some of the desired amalgam, for instance, tin-lead amalgam (about 3 grams), is also introduced 60 along with the mercury. This may be prepared by melting solder into the mercury, and heating, taking care to prevent the formation of oxides.

65 After the valve has been provided with its amalgam coating and the mercury along

with the amalgam has been placed within the valve, it is necessary to seal it hermetically in order to prevent the escape of the vaporized mercury when the apparatus is in use.

I prefer to seal the valve by means of a 70 welding operation, and I also take steps to avoid the permanent breaking down of the amalgam coating which would otherwise take place as a result of the welding operation.

When the valve is ready for sealing, I 75 drive a tapered plug 15 into the open end thereof, as shown in Fig. 2, until the tube is practically hermetically sealed, and I then saw this off even to the top of the valve, as indicated by the dotted line.

80 The valve is then placed within three-fourths of an inch of the top in water, and an oxy-acetylene flame is used to fuse over the entire end of the valve, after which two more layers of steel are added, as shown and indicated by the reference numerals 16 and 17, and thoroughly fused. While this end of the valve is red hot, it is turned upside down and the mercury and amalgam with the mercury is allowed to boil until the 85 boiling ceases. This applies amalgam to any part of the coating of the upper portion of the stem which may have broken down due to welding, and also to the end of the plug 15, so that when the valve has cooled, the amalgam coating will be intact. The method of sealing the valve and of applying the amalgam coating to the upper portion of the stem and the plug after sealing is described and forms the subject matter of claims in my 90 above-mentioned divisional application.

95 Another advantage of carrying on this welding process in conjunction with a water bath, as described above, in order to cause the hermetic sealing of the valve tube, is the avoidance of any possibility of the air within the valve body becoming so heated as the result of the heat of the welding operation, as to cause the blowing out of the plug, as the result of its expansion. The welding 100 may, of course, be effected electrically if desired.

105 I believe that I am correct in describing the metallic coatings herein as amalgams or alloys of mercury, but it will be understood that I also use the term "amalgam" herein not only specifically, but generally, to indicate the alloy or mixture of metals which are formed as a result of my improved methods of manufacture.

110 Tin and lead are known as tetrad metals, that is, they belong to a chemical series which forms the fourth group in the periodic classification table. Where the terms "tetrad metal" or "tin" are used in the claims it is 115 to be understood that they include not only tin but such equivalents as lead, or tin-lead.

120 While I have described herein some preferred embodiments of my invention, it will 125

of course be understood that many modifications and changes might be made by those skilled in the art without departing from the spirit or scope of my invention as defined by the appended claims.

What is claimed is as follows:

1. In a device of the kind described; a hollow metallic portion adapted to be exposed to high temperatures; a metallic working medium contained within said hollow portion which is capable of being vaporized at temperatures to which said hollow metallic portion is subjected when in use; and an intervening building up heat-transmitting medium on the inner wall of said hollow portion, said heat transmitting medium comprising metals common to said wall and to said working medium. 70
2. In a device of the kind described; a hollow portion of ferrous metal adapted to be exposed to high temperatures; a metallic working medium contained within said hollow portion which is capable of being vaporized at temperatures to which said hollow portion is subjected when in use; and an intervening heat-transmitting medium on the inner wall of said hollow portion, said heat transmitting medium comprising metals common to said ferrous metal wall and to said working medium. 75
3. In a device of the kind described, a hollow metallic portion adapted to be exposed to high temperature conditions; working mercury within said hollow portion; and an intervening heat-transmitting medium on the interior walls of said hollow portion, said medium comprising an amalgam containing iron. 80
4. In a device of the kind described, a hollow portion adapted to be exposed to high temperature conditions; a building up amalgam coating including iron and tin on the walls of said hollow portion; and working mercury contained within said hollow portion. 85
5. In a device of the kind described, a hollow portion adapted to be exposed to high temperature conditions; an amalgam coating including iron and a tetrad metal having building up properties; and working mercury contained within said hollow portion. 90
6. A body formed with a hollow portion adapted to be exposed to high temperatures; a metallic working medium contained within said hollow portion and capable of being vaporized at temperatures to which said hollow body is subjected when in use; and an intervening heat-transmitting medium on the inner wall of said portion, said medium containing a quantity of ferrous metal. 95
7. An engine valve formed with a hollow portion adapted to be exposed to high temperature conditions; an amalgam coating having building up properties on the walls of the hollow portion; said coating contain- 100

ing a ferrous metal and working mercury and an amalgam of said metal within said hollow portion.

8. A device of the kind described comprising a hollow metallic member adapted to be exposed to a high temperature and formed of different metals of varying heat conducting characteristics, the metal forming the interior walls of said hollow portion being an alloy of the metal forming the exterior walls of said portion. 105

In testimony whereof I affix my signature.  
THOMAS MIDGLEY, JR.

70

75

80

85

90

95

100

105

110

115

120

125

130